

July 25, 1950

I. R. KRAMER ET AL

2,516,125

ALLOY STEEL

Filed April 11, 1949

FIG 1



FIG 2



IRVIN R. KRAMER  
STEWART L. TOLEMAN  
WALTER T. HASWELL

Inventor

By

*S E Bush*

Attorney

## UNITED STATES PATENT OFFICE

2,516,125

## ALLOY STEEL

Irvin R. Kramer and Stewart L. Toleman, Washington, D. C., and Walter T. Haswell, Ligonier, Pa.

Application April 11, 1949, Serial No. 86,834

9 Claims. (Cl. 75—123)

(Granted under the act of March 3, 1883, as amended April 30, 1928; 370 O. G. 757)

1

The invention described herein may be manufactured and used by or for the Government of the United States of America for governmental purposes without the payment of any royalties thereon or therefor.

This invention relates to alloy steels and particularly to air-hardening alloy steels containing manganese and nickel.

This application is a continuation-in-part of our pending application, Serial No. 574,182, filed January 23, 1945, now abandoned.

It is well known that the optimum mechanical properties of steel are obtained when the steel has been first put in the martensitic condition and the martensite subsequently tempered. In other words, the best combination of strength and ductility is found in steels which have been tempered after first being heat treated to produce a martensitic structure. "Martensite" as used throughout this specification, is defined as the phase whose formation from austenite is dependent only on the lowering of temperature below a point (fixed by composition) called the  $M_s$  point and is thus independent of time (cooling rate).

The formation of martensite from a given quantity of austenite is predicated upon cooling said austenite to a low temperature within a certain critical period of time which is primarily also a function of composition. This critical cooling period, or reciprocally, the critical cooling rate, is that necessary to cool the steel to a relatively low temperature before the pearlite and pearlite-type reactions (producing soft products) have had time to begin. Thus, since the maximum cooling rate attainable in the center of a piece of steel is inherently limited by heat transfer factors, it is necessary to employ material having a proper alloy content if the soft-product reactions are to be inhibited for a sufficiently long period, and thus a large section of steel obtained in the fully hardened (martensitic) condition. Even though the cooling rate in the interior of a large section can, to a limited extent, be increased by rapid cooling (quenching) of the surface, this is not generally feasible due to the induced residual stresses attendant upon large differences in cooling rate between surface and center. Thus, from both the viewpoint of the limited maximum cooling rate attainable in the center of a large section and the viewpoint of minimizing differences in cooling rate between surface and center, it is necessary to use a composition having a very low critical cooling rate if a fully hardened, large-section product is to be obtained. For example, since the center of a 6-inch plate cooling in air cools from a temperature around  $1600^{\circ}$  F. at an average rate of about  $100^{\circ}$  F./hr., and that of an 18-inch plate at an average rate of about  $50^{\circ}$  F./hr., compositions

for fully hardenable plates of these dimensions must have, respectively, not greater critical cooling rates.

After hardening, it is necessary to temper the martensitic material to make it sufficiently ductile for practical use. As will appear below, phenomena associated with the tempering process may critically affect the properties of the finished product.

An air-hardening steel containing 2-6% manganese, together with a suitable tempering treatment therefor, is disclosed in a French patent issued in 1934 to the Societe Industrielle & Commerciale Des Aciers, and that patent represents the furthest prior advance in the art of air-hardening manganese steels of which we are aware.

The invention herein described also comprises an air-hardening steel containing 2-6% manganese and may be considered an improvement on the invention of the French patent.

It is the general object of this invention to provide a series of air-hardening manganese steels of improved mechanical properties.

It is another object to provide a series of manganese steels which may be fully hardened in large sections.

It is the particular object of the invention to provide a series of air-hardening manganese steels which will have, in large sections, excellent impact and ballistic properties after being fully-hardened and tempered, and will retain the properties for an indefinite period of time.

Other objects and advantages will in part be obvious and in part appear hereinafter.

This invention comprises a series of steel compositions, and includes particular embodiments, such as articles having one of these compositions, wherein the utility of the composition becomes operative. The steels of this invention contain, among other components, manganese in quantities from 2-6 percent. It should be pointed out that these limitation are not arbitrary, but are related to the recognized classification of manganese steels. Manganese steels containing less than 2% Mn are classified as pearlitic steels and constitute a well established group of structural materials, e. g. the S. A. E. 1300 series containing 1.60 to 1.90% Mn. On the other hand, if more than 6% Mn is present the material begins to approach the Hadfield austenitic steels in composition. Substantial quantities of retained austenite will exist at room temperature and further cooling will be necessary to attain the fullest possible formation of martensite. Of course the 6% figure is not absolute, and due to factors such as stabilization, a small quantity (about 1-5%) of retained austenite may exist at room temperature in our steels, but nevertheless they will be "fully

hardened" in the sense that no more martensite is formed even on cooling to liquid air temperatures.

In steels containing other elements in alloying proportions the limits set for the quantity of manganese alone may not be controlling of the classification of the steel, i. e. the nature of the austenite transformation product. Therefore, if a fully hardened material is to be obtained in large sections upon air cooling it is necessary to specify composition in terms of a factor based upon all of the alloying components present. We call this factor the "manganese equivalent" and it will be quantitatively defined hereinafter. By "alloying component" is meant a component which, by virtue of its inherent nature and of the quantity of it present, relative to the overall composition, substantially affects the austenite transformation. It is to be distinguished from components which merely affect properties of the transformation product, or merely facilitate fabrication, or are present unintentionally. Thus, while in some steels molybdenum, silicon and chromium substantially effect austenite transformation, here whatever effect they exert is masked by the more powerful influence of manganese and nickel, and they are not alloying components in the steels of this invention.

It should be pointed out that neither a 2% Mn content in a straight manganese steel, nor a 2% "manganese equivalent" in a complex alloy steel, will produce a fully hardened structure on slow (air) cooling, but rather a partially pearlitic structure. Note that insofar as the French patent teaches equivalency in this respect throughout the 2-6% range of manganese content, its teaching is contradicted. We have found a way to define an alloy composition which permits manganese to be as low as 2% and still produces a fully hardened material in large sections upon slow cooling, and which at the same time (and this is even more important) eliminates a peculiar detrimental effect of tempering said material.

It has been found that upon tempering the martensitic structure formed with a straight manganese steel sufficiently to induce reasonable ductility, viz. at from about 550° C. (1022° F.) to about 675° C. (1245° F.) for from about 2 hours to about 4 hours, a substantial quantity (roughly 10-30%) of austenite is formed; and that upon cooling to room temperature after tempering, this austenite decomposes to form a product which has a very detrimental effect upon the impact properties of the steel.

The X-ray data establish that this product is an alpha phase. It can be either bainite or martensite. It is, of course, obvious that the chemical composition of the temper-formed austenite will be different from that of the original matrix austenite from which the martensite was first formed. Accordingly, the respective austenite-martensite reactions will be different. The formation of austenite on tempering, and its decomposition to an alpha constituent on cooling is shown by the X-ray data in Table I, the water quenched "W. Q." specimens showing the phases present at the tempering temperature and the furnace cooled "F. C." those present after (slow) cooling from the tempering temperature. The specimens are a 3.66% Mn, 0.11% C steel (note the similarity to one of the examples given in the French patent) austenitized at 900° C. (1650° F.) furnace-cooled at a rate corresponding to that at the center of a 6-inch plate, and tempered at 650°

C. to (1200° F.) and taken to room temperature as indicated:

Table I

| 5  | Tempering time | X-ray diffraction lines |                        | Charpy impact |
|----|----------------|-------------------------|------------------------|---------------|
|    |                | $\alpha$ sharp          | $\gamma$ fairly strong |               |
| 10 | 4 hrs. W. Q.   | $\alpha$ sharp          | $\gamma$ fairly strong | Ft.-lbs.      |
|    | 16 hrs. W. Q.  | do                      | $\gamma$ strong        |               |
|    | 4 hrs. F. C.   | $\alpha$ broad          | $\gamma$ medium        |               |
|    | 16 hrs. F. C.  | $\alpha$ very broad     | $\gamma$ faint         |               |

The gamma line, of course, proves the presence of austenite and the broad alpha line, the presence of the decomposition product. The impact properties of the furnace-cooled specimens (in which the austenite has had time to decompose) are much lower than those of the water quenched specimens. Thus, it might appear that simply by quenching, the unfavorable effect of decomposition of this temper-formed austenite could be overcome. However, this is not the case because of the fact that the austenite "retained" upon quenching the tempered straight manganese steels also decomposes in time (beginning in about 7 to 14 days) to produce an equally brittle product. And further, in a section larger than about 2 inches, it is not possible by quenching to even temporarily forestall the decomposition of the austenite forming on tempering. The effect of "standing time" on temper-formed austenite was determined for three manganese steels and is shown in Table II. The steels were slowly cooled from austenitizing temperature, tempered at about 600° C. (1110° F.) and water-quenched from tempering temperature. X-ray data were taken within 24 hours of heat treatment and again after approximately 8 months.

Table II

| 40 | Alloy | Mn   | C    | Mo    | Si   | Gamma line    |            |
|----|-------|------|------|-------|------|---------------|------------|
|    |       |      |      |       |      | 24 hrs.       | 8 months   |
| 45 | MCC   | 3.38 | 0.16 | 0.99  | 0.14 | fairly strong | none       |
|    | MCA   | 4.67 | 0.16 | ----- | 0.20 | do            | very faint |
|    | MBV   | 4.16 | 0.15 | 0.04  | 0.03 | do            | trace      |

It is necessary to point out that this austenite formation on tempering is not to be confused with "temper-brittleness" since the latter phenomenon sometimes occurs as a result of operational steps similar to those bringing about the former. Temper-brittleness is a widely recognized phenomenon, has been extensively investigated, and is now generally accepted as being due to the formation of a special precipitate such as carbide, nitride or oxide. See Hollomon, "Temper Brittleness" 36 Trans. A. S. M. 473, (1946). It will be apparent to those skilled in the art that the austenite formation, proven here by X-ray data, could only occur in a steel having an  $A_1$  critical temperature low enough (alloy content high enough) to fall into the tempering temperature region.

65 It has been found, and herein lies the most important aspect of the invention, that the addition of nickel to the manganese steels, in requisite amounts, forestalls indefinitely the breakdown of the temper-formed austenite, with either slow or rapid cooling (and thus in any section size) after tempering, and makes possible the production of a tempered manganese steel having high impact toughness.

70 Further, it has been found that nickel (in any quantity) has an effect on the critical cooling

rate about half as strong as that of manganese, and thus, by use of appropriate amounts, can be substituted for manganese, simply from the point of view of obtaining a fully hardened structure in large sections. Thus we define "manganese equivalent" as the total manganese content plus one-half of the nickel content.

With regard to the relation of nickel content to impact properties of the tempered material it has been found, as will be seen from Table III, that nickel has a disproportionately weak effect toward stabilizing the temper-formed austenite in quantities less than 1%.

Table III

| Alloy | Ni content | Charpy V-Notch | Brinell Hardness |
|-------|------------|----------------|------------------|
| MVK   | 0          | 47             | 260              |
| MEC   | .83        | 55             | 266              |
| MEB   | 1.16       | 67             | 275              |
| MEA   | 1.68       | 76             | 272              |
| MDS   | 2.24       | 120            | 270              |

  

| Composition | C    | Mn   | Ni   | Mo   | Si   | "Mn" Equiv." |
|-------------|------|------|------|------|------|--------------|
| MVK         | 0.11 | 3.66 | 0    | 0.89 | 0.14 | 3.7          |
| MEC         | .26  | 3.64 | .83  | 0.30 | 0.17 | 4.1          |
| MEB         | .26  | 3.68 | 1.16 | 0.28 | 0.17 | 4.3          |
| MEA         | .26  | 3.25 | 1.68 | 0.30 | 0.17 | 4.1          |
| MDS         | .08  | 2.75 | 2.24 | 0.61 | 0.05 | 3.9          |

From about 1% to about 2.5% nickel, there is a continuous improvement in impact properties with nickel content. Above that limit it would appear that the austenite is completely stabilized and no further improvement in impact properties is observed. The nickel above 2.5%, however, is still operative to increase the "hardenability" of the steel in accordance with the definition of the manganese equivalent, and thus the overall composition is defined to permit nickel as high as 8%, this limit being fixed by the manganese equivalent and minimum manganese content limitations.

It may be of interest to point out that a second tempering treatment, usually performed at a temperature somewhat below that of the first, brings about some improvement in impact properties in the manganese-nickel steels.

Carbon has a weak effect on the properties of these steels within the range from about 0.05% to about 0.30%. If less than 0.05% C is present the steel will not form hard martensite. If more than 0.30% is present, some carbides will form on cooling which have a detrimental effect on impact as well as other properties. The effect of carbon on "hardenability" is appreciable only in sections having a relatively low hardenability (low manganese equivalent) as seen from the accompanying drawing, Fig. 1. As will also be seen from Fig. 1 the manganese equivalent must be at least 3.5 to get a martensitic structure in even a  $\frac{1}{2}$ -inch section and must be 4 or a little greater to get a fully hardened large section article. As was stated above, if the manganese equivalent is greater than 6 excessive austenite will be retained on cooling to room temperature in the initial hardening operation. By holding the manganese equivalent between 4 and 6, it is possible to fully harden articles up to 18 inches in maximum section size.

Molybdenum may be added to our Fe-Mn-Ni alloy to form a preferred embodiment of the in-

vention. It is found to raise the tensile strength of the final product without detracting from other properties. This finding is believed merely to confirm the teaching of the French patent since the molybdenum here apparently performs the same function as therein disclosed, viz. simply improvement in mechanical properties. Its effect is more or less continuous up to about 0.50-0.75%. It is interesting to point out that while molybdenum is known to have a beneficial effect in overcoming temper-brittleness, it has no such effect on the tempering phenomenon observed here. As a matter of preferred practice, molybdenum is added to most of the steels made in accordance with this invention, but it is not an "alloying component" as that term is hereinbefore defined. Similarly, silicon is present in these alloys simply because it is inherent in good steel-making practice. Its use in the quantities shown is determined simply by practice well known in the art and not related to the invention. In Table IV below are given general mechanical properties for a few of the Ni-Mn steels of this invention. In addition to the analysis given, each steel contains quantities of molybdenum and silicon as set out above. The steels were all fully hardened by slow cooling from an austenitizing temperature of 900° C. (1650° F.) and tempered at 600° C. (1112° F.) for 4 hours.

Table IV

| Alloy       | T. S.    | Y. S.    | Per Cent | Per Cent |
|-------------|----------|----------|----------|----------|
|             |          |          | Elong.   | Red. of  |
|             | P. s. i. | P. s. i. | 2 inch   | Area     |
| MKP 3.42 Mn |          |          |          |          |
| 1.55 Ni     | 121,500  | 93,300   | 22       | 63       |
| 0.11 C      |          |          |          |          |
| 1.70 Ni     | 120,000  | 77,000   | 23       | 66       |
| MKR 3.33 Mn |          |          |          |          |
| 0.17 C      | 116,000  | 79,000   | 25.2     | 62.9     |
| MGK 3.47 Mn |          |          |          |          |
| 1.47 Ni     | 112,000  | 95,000   | 29.3     | 75       |
| 0.20 C      |          |          |          |          |
| 1.53 Ni     | 126,000  | 82,000   | 27       | 58       |
| MKS 3.52 Mn |          |          |          |          |
| 0.08 C      | 118,000  | 107,000  | 28       | 62       |
| MCT 2.73 Mn |          |          |          |          |
| 1.93 Ni     | 112,000  | 67,500   | 29       | 61       |
| 0.22 C      |          |          |          |          |
| 2.24 Ni     | 120,000  | 100,000  | 27       | 58       |
| MDO 2.72 Mn |          |          |          |          |
| 0.19 C      | 118,000  | 107,000  | 28       | 62       |
| MDV 2.85 Mn |          |          |          |          |
| 2.35 Ni     | 112,000  | 67,500   | 29       | 61       |
| 0.17 C      |          |          |          |          |

The teaching of the French patent in regard to improvement in mechanical properties by additions of vanadium also applies to the improved material of this invention, but in such a remarkable way that it seems desirable to give specific examples. The effect is clearly seen by comparison of the steels MML (3.20 Mn, 160 Ni, 0.60 Mo, 0.17 Si and 0.13 C) and MMK (4.05 Mn, 1.74 Ni, 0.60 Mo, 0.17 Si, 0.13 C and 0.19 V). Thus, after austenitizing at 900° C. (1650° F.), cooling, and tempering for 8 hours at: (a) 600° C. (1112° F.), (b) 550° C. (1030° F.) and (c) 500° C. (930° F.) the properties given in Table V were obtained.

Table V

|     |     | Tensile Strength | Yield   | Percent Elong. 2 inch | Percent of Red. of Area |
|-----|-----|------------------|---------|-----------------------|-------------------------|
| (a) | MML | 126,250          | 108,000 | 31                    | 65                      |
|     | MMK | 171,700          | 148,500 | 21                    | 58                      |
| (b) | MML | 138,500          | 123,000 | 20                    | 57                      |
|     | MMK | 178,000          | 161,000 | 19.5                  | 53                      |
| (c) | MML | 163,000          | 146,500 | 19.5                  | 56.5                    |
|     | MMK | 160,050          | 151,500 | 21.7                  | 67.2                    |

In Table VI below are given compositions of some other Mn-Ni-V steels which have been prepared.

Table VI

| Alloy | Mn   | Ni   | Mo  | Cr  | Si  | C   | V   |
|-------|------|------|-----|-----|-----|-----|-----|
| MHU   | 3.48 | 1.52 | .28 | .24 | .13 | .17 | .07 |
| MLD   | 3.68 | 1.51 | .29 | —   | .40 | .09 | .21 |
| MLW   | 3.50 | 1.74 | .25 | —   | .16 | .25 | .18 |
| MLX   | 3.39 | 1.66 | .49 | —   | .14 | .25 | .19 |
| MLY   | 3.32 | 1.67 | .83 | —   | .14 | .27 | .18 |
| MMD   | 3.55 | 1.59 | .59 | —   | .05 | .13 | .18 |
| MME   | 3.48 | 1.57 | .49 | —   | .04 | .24 | .18 |
| MMK   | 4.05 | 1.74 | .60 | —   | .17 | .13 | .19 |
| MMAD  | 3.20 | 2.22 | .53 | .20 | .46 | .26 | .22 |

Table VII shows the ordinary properties of some of these alloys with indicated tempering treatment after austenitizing at 900° C. (1650° F.) and slowly cooled.

Table VII

| Alloy | Tempered              | T. S.   | Y. S.   | Percent Elong. | Percent R. A. | TS/Y.S. | Charpy V-notch |
|-------|-----------------------|---------|---------|----------------|---------------|---------|----------------|
| MHU   | 930° F.—8 hrs. W. Q.  | 151,000 | 128,750 | 18.0           | 53.5          | 85      | 31             |
| MHU   | 1110° F.—8 hrs. W. Q. | 131,000 | 107,750 | 21.0           | 61.0          | 82      | 97             |
| MLD   | 930° F.—8 hrs. W. Q.  | 147,750 | 122,500 | 22.0           | 64.0          | 83      | 27             |
| MLD   | 1110° F.—8 hrs. W. Q. | 135,750 | 118,750 | 23.0           | 69.6          | 87      | 106            |
| MLW   | 930° F.—8 hrs. W. Q.  | 181,000 | 150,000 | 13.0           | 33.0          | 85      | 10             |
| MLW   | 1110° F.—8 hrs. W. Q. | 162,000 | 136,000 | 16.8           | 42.2          | 84      | 59             |
| MLX   | 930° F.—8 hrs. W. Q.  | 192,000 | 163,000 | 15.0           | 43.0          | 85      | 13             |
| MLX   | 1100° F.—8 hrs. W. Q. | 174,000 | 150,000 | 15.3           | 34.0          | 86      | 49             |
| MLY   | 930° F.—8 hrs. W. Q.  | 200,200 | 179,000 | 15             | 39.0          | 89      | 17             |
| MLY   | 1110° F.—8 hrs. W. Q. | 172,000 | 147,000 | 18.5           | 49.5          | 86      | 20             |

Table VIII shows the mechanical properties of two other Mn-Ni-V steels tested at an elevated temperature, viz 500° C. (930° F.). Note that these specimens received a double tempering treatment before testing.

Table VIII

| Alloy | Tempering Treatment                           | T. S.   | Y. S.   | Percent Elong. | Percent R. A. |
|-------|-----------------------------------------------|---------|---------|----------------|---------------|
| MMD   | 1200° F.—8 hrs. F. C. + 1022° F.—8 hrs. F. C. | 80,000  | 75,000  | 35             | 76            |
| MMD   | 1112° F.—8 hrs. F. C. + 1022° F.—8 hrs. F. C. | 115,000 | 116,000 | 25             | 46            |
| MMD   | 932° F.—8 hrs. F. C. + 932° F.—8 hrs. F. C.   | 125,000 | 118,000 | 32             | 71            |
| MME   | 1112° F.—8 hrs. F. C. + 1022° F.—8 hrs. F. C. | 100,000 | 83,000  | 35             | 78            |
| MME   | 1112° F.—8 hrs. F. C. + 1022° F.—8 hrs. F. C. | 110,000 | 103,000 | 22             | 35            |
| MME   | 932° F.—8 hrs. F. C. + 932° F.—8 hrs. F. C.   | 136,000 | 115,000 | 30             | 72            |

Two other Mn-Ni-V steels were given stress-rupture tests, the stresses required to cause rupture in 1000 hours at the indicated temperatures being determined as shown in Table IX. Since it is suggested that these steels could be used for applications such as turbine rotors, comparative data are given for two rotor steels, "AAC" and "ZR," now used for turbine rotors.

Table IX

| Alloy | Heat Treatment                                 | Testing Temperature | Stress          |
|-------|------------------------------------------------|---------------------|-----------------|
| AAC   | Normalized                                     | 830° F.             | P. s. i. 65,000 |
| AAC   | do                                             | 930° F.             | 47,000          |
| ZR    | do                                             | 830° F.             | 55,000          |
| MMAD  | 1650° F.—F. C.—Tempered twice at 932° F.—F. C. | 650° F.             | 155,000         |
| MMAD  | do                                             | 850° F.             | 95,000          |
| MMAD  | do                                             | 950° F.             | 55,000          |
| MMK   | do                                             | 650° F.             | 152,000         |
| MMK   | do                                             | 850° F.             | 92,000          |
| MMK   | do                                             | 950° F.             | 52,000          |

An important element which bears critical relation to this invention and must be given special consideration in this specification is chromium.

Contrary to the effect of this element in alloy steels generally, and contrary to the suggestion of the French patent, it has been found that chromium has a distinctly detrimental effect on the impact properties of these steels, and at the same time contributes only slightly to the tensile properties of the material. Chromium has been found to accelerate the breakdown of the aforementioned temper-formed austenite. Thus, if pure ferrous material (ingot iron) is available, its use is recommended and chromium should be entirely avoided. In industrial practice, of course, it is necessary to use scrap as a partial source of iron and thus it is practically impossible to make a heat of commercial steel without from about 0.1% to about 0.3% residual chromium. Fortunately, however, it has been found that by the simple expedient of raising the minimum nickel content in rough proportion to the amount of chromium present the detrimental effect of the

latter element will be overcome. Of course the amount of residual chromium which will occur in the finished product must be estimated in advance, or determined from analysis of the melt, in order that the minimum nickel content neces-

sary to insure against decomposition of the temper-formed austenite will be known. It has been found that some increase above the minimum nickel content of 1% should be specified if anything but ingot iron (or equivalent) is used as a base metal for the alloys, and that if as much as 0.1% chromium occurs this increase should amount to about 0.4 to about 0.5% nickel. Chromium up to 0.30%, which should be about the maximum residual from scrap pick up, may be tolerated if at least 2.25% nickel is present (1.25% above the minimum for non-chromium steels). Thus, it is necessary with chromium-bearing steels to add nickel over and above the 1% lower limit in quantities roughly about four times the total chromium content. In such case, of course, the manganese content must be adjusted to provide a given desired manganese equivalent. The data in Table X demonstrate the detrimental effect of chromium and the manner in which it may be overcome by increasing the nickel content as set forth above. The data in Table X are from steels austenitized at 900° C. (1650° F.) and slowly cooled, then tempered at 600° C. (1110° F.) for 4 hours and water quenched. Note that water quenching did not forestall the

breakdown of austenite in the non-nickel bearing steels of section size necessary for these specimens (described below) long enough for the test to be made.

Table X

|       | Mn   | Ni   | Mo   | Cr    | Si   | C    | Fracture          | Limit Velocity | Charpy V-notch Impact |
|-------|------|------|------|-------|------|------|-------------------|----------------|-----------------------|
| MKS   | 3.32 | 1.63 | 0.47 | ----- | 0.25 | 0.14 | Fibre             | 3,600          | 145                   |
| MKR   | 3.33 | 1.70 | 0.27 | ----- | 0.11 | 0.17 | do                | 3,600          | 140                   |
| MKP   | 3.42 | 1.55 | 0.28 | ----- | 0.35 | 0.11 | do                | 3,600          | 105                   |
| WNY-3 | 3.63 | 1.42 | 0.45 | 0.18  | 0.32 | 0.12 | Brittle and Fibre | 3,420          | 67                    |
| MGC   | 3.65 | 1.50 | 0.26 | 0.25  | 0.08 | 0.17 | Brittle           | 3,300          | -----                 |
| MGP   | 3.58 | 1.60 | 0.23 | 0.41  | 0.16 | 0.17 | do                | 2,800          | 45                    |
| MM    | 2.79 | 2.28 | 0.52 | 0.30  | 0.14 | 0.11 | Fibre             | 3,500          | -----                 |
| MMN   | 3.17 | 2.29 | 0.50 | 0.29  | 0.14 | 0.11 | do                | 3,460          | 124                   |
| MMO   | 3.17 | 2.42 | 0.29 | 0.27  | 0.28 | 0.23 | do                | 3,450          | -----                 |
| MMP   | 3.50 | 2.41 | 0.50 | 0.23  | 0.28 | 0.23 | do                | 3,440          | -----                 |

Figure 2 shows comparative limit-velocity values at a varying Brinell hardness for a typical alloy (nominal composition: 3.5% Mn, 2.5% Ni, 0.12% C) of this invention and for an acceptable armor plate. Thus, the dashed line is a plot of limit-velocity versus hardness for our steel, and the solid line (A) is such a plot for an acceptable armor plate 1 1/4 inches in thickness. Varying hardnesses were developed by different tempering treatments. The points, "B" and "C," represent, respectively, single tests in the as-received condition of specimens cut from the center of a 12-inch and an 18-inch plate of acceptable armor plate. "Limit-velocity" is used here as meaning the velocity of a .50 caliber bullet required to just "shoot off" a finger 2 1/2 inches long and 1 1/2" x 1 1/2" square, notched 1/8" at its base.

It will be understood that the examples herein described are illustrative only and that the invention is not to be limited except as defined by the herewith appended claims.

What is claimed is:

1. An alloy steel comprising essentially from about 0.05% to about 0.30% carbon, from about 2% to about 6% manganese, from about 1% to about 8% nickel, balance iron and incidental impurities, and having a manganese equivalent between 3.5 and 6, the nickel content of said alloy steel being further limited in that it is at least 1% plus about four times the residual chromium content.

2. An alloy steel comprising essentially from about 0.05% to about 0.30% carbon, from about 2% to about 6% manganese, from about 2.25% to about 8% nickel, balance iron and incidental impurities, and having a manganese equivalent between 3.5 and 6, said alloy steel containing from traces to about 0.3% chromium.

3. An alloy steel consisting essentially of from about 0.05% to about 0.30% carbon, from about 2% to about 6% manganese, from about 1% to about 8% nickel, from about 0.01% to about 0.3% silicon, from about 0.01% to about 0.7% molybdenum, balance substantially all iron plus residual quantities of elements commonly present in steel but containing no measurable quantity of chromium, and having a manganese equivalent between 3.5 and 6.

4. An alloy steel consisting essentially of from about 0.05% to about 0.30% carbon, from about 2% to about 6% manganese, from about 1% to about 8% nickel, from about 0.01% to about 0.3% silicon, from about 0.01% to about 0.7% molybdenum, balance substantially all iron plus residual quantities of elements commonly present in steel, and having a manganese equivalent between 3.5 and 6, the nickel content of said alloy

steel being further limited in that it is at least 1% plus about four times the residual chromium content.

5. An alloy steel consisting essentially of from

about 0.05% to about 0.30% carbon, from about 2% to about 6% manganese, from about 1.5% to about 8% nickel, from about 0.01% to about 0.3% silicon, from about 0.01% to about 0.7% molybdenum, balance substantially all iron plus residual quantities of elements commonly present in steel, and having a manganese equivalent between 3.5 and 6, and containing from traces to about 0.1% residual chromium.

6. An alloy steel consisting essentially of from about 0.05% to about 0.30% carbon, from about 2% to about 6% manganese, from about 2.25% to about 8% nickel, from about 0.01% to about 0.3% silicon, from about 0.01% to about 0.7% molybdenum, balance substantially all iron plus residual quantities of elements commonly present in steel, and having a manganese equivalent between 3.5 and 6, and containing from about 0.1% to about 0.3% residual chromium.

7. A slow-cooled, fully hardened steel article from about 2 inches to about 18 inches in maximum section size having a chemical composition at defined in claim 1 and further limited chemically in that the manganese equivalent within the limits recited is approximately proportional to the section size within the limits recited.

8. A slow-cooled, fully hardened, tempered steel article from about 2 inches to about 18 inches in maximum section size having a chemical composition as defined in claim 1 and further limited chemically in that the manganese equivalent within the limits recited is approximately proportional to the section size within the limits recited, said steel article being characterized by high impact strength.

9. A slow-cooled, fully hardened, tempered steel article from about 2 inches to about 18 inches in maximum section size having a chemical composition as defined in claim 1 and further limited chemically in that the manganese equivalent within the limits recited is approximately proportional to the section size within the limits recited, said steel article being characterized by the absence of decomposition products of tempered austenite.

IRVIN R. KRAMER.  
STEWART L. TOLEMAN.  
WALTER T. HASWELL.

REFERENCES CITED

The following references are of record in the 70 file of this patent:

FOREIGN PATENTS

| Number  | Country       | Date         |
|---------|---------------|--------------|
| 768,468 | France        | Aug. 7, 1934 |
| 440,894 | Great Britain | Jan. 8, 1936 |